

# UNITED STATES PATENT OFFICE.

LAWRENCE ADDICKS, OF CHROME, NEW JERSEY.

## PROCESS FOR MAKING BRASS.

1,041,940.

Specification of Letters Patent. Patented Oct. 22, 1912.

No Drawing.

Application filed January 12, 1911. Serial No. 602,154.

To all whom it may concern:

Be it known that I, LAWRENCE ADDICKS, a citizen of the United States, residing at Chrome, in the county of Middlesex and State of New Jersey, have invented certain new and useful Improvements in the Process for Making Brass, of which the following is a specification.

My invention relates to a new and improved process for making brass.

It relates particularly to a process for making brass much more economically than it is made at present and on a much larger scale.

The method at present in vogue in manufacturing brass is as follows: In a crucible holding approximately 100 lbs. there is melted a charge of copper and a certain proportion of brass scrap and spelter. The copper having been thus melted, the zinc is introduced, the charge being then skimmed and poured as rapidly as possible, in order to avoid loss of the zinc which volatilizes very rapidly at the temperature of molten copper. This method of manufacture is very expensive, since the cost of the crucibles is high, the depreciation rapid and the breakage very considerable. Moreover, in this method, the brass is produced on a small scale, and the labor cost is excessive. To overcome certain of these disadvantages it has been proposed to make the brass in a reverberatory furnace, but, so far as I am aware, without success. This lack of success is due in the first place to the very great loss of zinc, and, secondly, to the difficulty of maintaining a uniform grade in the brass produced. A uniform grade is necessary, in order to assure a uniform color in the product.

The object of my invention is to overcome the obstacles that have stood in the way of using the reverberatory furnace, or a similar large source of heat, and to produce the brass on a large scale and at a price for labor not much exceeding the casting of copper ingots by the copper founder.

To carry out my invention, I melt in a reverberatory furnace, or similar source of heat, a full charge of copper such as is put into the furnace by the copper melters. The size of these charges varies from 20 to 250 tons per twenty-four hours, and the method is in no way changed from ordinary copper melting. Into the furnace are placed copper cathodes, or copper in the shape of

ingots, or in any form desired, and the same are reduced to the molten state. I now provide an intermediate ladle, such, for instance, as the ordinary back gear crane ladle in common use in foundries, suitably lined with fire-clay. A convenient size for the intermediate ladle will be a capacity of two or three tons. I draw into the intermediate ladle a fraction of the furnace charge, and introduce thereto the desired quantity of zinc, quickly incorporating it into the copper. The two or three tons of brass are then promptly drawn off from the ladle and cast into ingots, or other desired shapes.

It is evident that the molten copper will be delivered to the ladle at no greater cost than to the molds in which copper ingots are cast, and that, therefore, the entire cost of making the brass will be simply the cost of materials, plus whatever zinc loss is involved, plus the ladling cost, which will be little more than that of ladling the original copper ingots. I can, of course, from one furnace charge, produce a different brass composition in each intermediate ladle charge, by changing the relative proportions of the copper and zinc put into the ladle.

My invention thus eliminates entirely a large part of the present brass founding cost. The exact quantity that can be handled to advantage at a time will be largely determined by the loss of zinc that is encountered, and this quantity of copper can be regulated within quite wide limits, according to circumstances, but a suitable amount will be found to be from one to three tons. It is evident that any suitable and convenient source of heat may be used, the only condition for working rapidly and on a large scale being that said heat source shall be capable of melting large amounts of copper at one charge.

By the term "brass" as used herein is meant any alloy of copper and zinc, with or without the addition of other metals; and thus includes for example German silver, and high brasses, sometimes called bronzes.

Having thus fully described my process and the manner in which it is to be carried out, what I claim is:—

1. The process of manufacturing brass, which consists in melting a large quantity of copper by a suitable source of heat, drawing off a fraction of the molten copper into a suitably lined intermediate receptacle, add-

ing to the said receptacle the proper percentage of zinc, and casting the resulting brass into the desired shape.

2. The process of manufacturing brass, which consists in reducing to the molten state by a suitable source of heat a relatively large mass of copper, transferring to an intermediate receptacle successive charges of molten copper approximating 10 two to three tons each, adding to each charge

the desired percentage of zinc, and casting the resulting brass to the desired shape.

In witness whereof, I have hereunto signed my name in the presence of two subscribing witnesses.

LAWRENCE ADDICKS.

Witnesses:

C. W. DEACON,  
E. J. BULFIN.